

## UNITED STATES PATENT OFFICE

2,130,242

## VULCANIZATION OF RUBBER

William E. Messer, Cheshire, Conn., assignor to  
United States Rubber Products, Inc., New  
York, N. Y., a corporation of Delaware

No. Drawing. Application February 16, 1935,  
Serial No. 6,807

## 2 Claims. (Cl. 18—53)

This invention relates to the use of new and improved accelerator combinations, useful in the production of vulcanized rubber goods.

An object of this invention is to provide a new activator for organic accelerators and more particularly for thiazyl sulphide vulcanization accelerators such as the arylene thiazyl sulphides and disulphides which when used in conjunction therewith will tend to produce less scorching and better calendering as well as better ageing rubber stocks.

These activators are characterized in being broadly amino thiophenols characterized by the grouping

15



20 wherein R is hydrogen or a substituted element or group. Examples are o-amino thiophenol, o-o' diamino-diphenyl disulphide, o-o' diamino-diphenyl monosulphide, p-amino thiophenol, p-p' diamino-diphenyl monosulphide, m-amino thiophenol, m.m'-diamino-diphenyl disulphide, m.m'-diamino diphenyl monosulphide, o-p'-diamino diphenyl disulphide, o-p'-diamino diphenyl sulphide and halogen and/or alkyl nuclear-substituted derivatives thereof. The salts 25 and acyl derivatives of the amino thiophenols may also be used, as where the hydrogen of the sulphydryl group is replaced by metal or an acyl group.

30 The following example is given to illustrate preferred aspects of the invention and is not to be construed as limiting thereof. The parts given are parts by weight. T stands for tensile in pounds per square inch at break, and E stands for percent elongation at break. The stock that 35 is tested for scorching properties, and tensiles before and after ageing is a tire tread stock.

## Example 1

| 45                                    | Stock  | Parts  |   | 50 |
|---------------------------------------|--------|--------|---|----|
|                                       |        | A      | B |    |
| Smoked sheets.....                    | 100.00 | 100.00 |   |    |
| Carbon black.....                     | 42.00  | 42.00  |   |    |
| Zinc oxide.....                       | 10.00  | 10.00  |   |    |
| Pine tar.....                         | 3.50   | 3.50   |   |    |
| Sulphur.....                          | 3.25   | 3.25   |   |    |
| Zinc soap of cocoanut oil acids.....  | 4.00   | 4.00   |   |    |
| Mercaptobenzothiazole.....            | 1.25   | .30    |   |    |
| o-o' diamino diphenyl disulphide..... |        | .90    |   |    |

## Scorch test (5 pounds per sq. in. steam pressure)

| Cure in minutes | A    |     | B    |     | 5 |
|-----------------|------|-----|------|-----|---|
|                 | T    | E   | T    | E   |   |
| 75.....         | 1665 | 745 | 1017 | 795 |   |
| 80.....         | 2527 | 817 | 1692 | 802 |   |
| 90.....         | 2760 | 782 | 2107 | 817 |   |

10

## Unaged

| Cure in mins. at 30 lbs. sq. in. steam pressure | A    |     | B    |     | 15 |
|-------------------------------------------------|------|-----|------|-----|----|
|                                                 | T    | E   | T    | E   |    |
| 20.....                                         | 3910 | 703 | 2820 | 676 |    |
| 30.....                                         | 3970 | 643 | 3960 | 703 |    |
| 40.....                                         | 4100 | 603 | 4400 | 690 |    |
| 50.....                                         | 4680 | 623 | 4530 | 673 | 20 |
| 60.....                                         | 4510 | 600 | 4610 | 666 |    |

## Aged 24 hrs. at 212° F.

|         |      |     |      |     |    |
|---------|------|-----|------|-----|----|
| 20..... | 3636 | 406 | 3780 | 495 | 25 |
| 30..... | 3197 | 365 | 3815 | 425 |    |
| 40..... | 3685 | 365 | 3790 | 445 |    |
| 50..... | 3265 | 380 | 2755 | 360 |    |
| 60..... | 2780 | 345 | 3430 | 440 |    |

Aged 168 hrs. in oxygen bomb (300 pounds 30  
oxygen maintained at 60° C.)

|         |      |     |      |     |    |
|---------|------|-----|------|-----|----|
| 20..... | 1060 | 605 | 1567 | 567 |    |
| 30..... | 1895 | 565 | 1825 | 557 |    |
| 40..... | 1693 | 452 | 1737 | 510 |    |
| 50..... | 1472 | 452 | 1592 | 475 | 35 |
| 60..... | 1210 | 385 | 1412 | 412 |    |

It will be observed that the initial cure, as shown by the scorch test, is retarded by use of the combination in B. Also that the optimum cure is reached at about the same time as with the full amount of mercaptobenzothiazole (stock A) which shows that an economy in use of the thiazole accelerator may be obtained by the present invention and further with an improvement in ageing properties. 40

Instead of mercaptobenzothiazole, its disulphide, mercapto-benzo-thiazole-disulphide (di-benzothiazyl disulphide) may be used, as well as other well known thiazole accelerators which are 50 derivatives, substitution products or salts of mercaptobenzothiazole illustrated by dinitro phenyl ester of mercaptobenzothiazole, benzoyl benzothiazyl sulphide, etc.

The amount of activator usable may vary from 55

that specifically shown. Generally it is usable in the same proportions as prior art activators of organic accelerators. The term rubber is to be construed broadly as including caoutchouc, balata, gutta percha, rubber isomers, synthetic rubber, and is applicable to latex whether naturally occurring or artificially preferred.

5 The activators may be used with different types of stock than that illustrated, with other compounding ingredients and other proportions of ingredients. In the case of white stocks the activator is substantially non-discoloring which is another attribute of this invention.

Having thus described my invention, what I 10 claim and desire to protect by Letters Patent is:

1. A process of producing vulcanized rubber goods which comprises accelerating the vulcanization of a vulcanizable rubber stock with an arylene thiazyl sulphide accelerator and an added

amount of an activator therefor having the general formula



5

where R is H or the grouping within the parenthesis the proportion of activator being greater than the proportion of the sulphide accelerator. 10

2. A process of producing a vulcanized rubber product which comprises incorporating in rubber prior to vulcanization a vulcanizing agent, an arylene thiazyl sulphide accelerator and a substantially pure diamino-diphenyl sulphide in 15 which the proportion of the diphenyl sulphide preponderates over the proportion of the sulphide accelerator.

WILLIAM E. MESSER.